

# UNITED STATES PATENT OFFICE.

OSWALD SILBERRAD, OF BLACKHEATH, ENGLAND.

## EXPLOSIVE.

No. 849,925.

Specification of Letters Patent

Patented April 9, 1907.

Application filed September 27, 1906. Serial No. 336,460.

*To all whom it may concern:*

Be it known that I, OSWALD SILBERRAD, a subject of the King of Great Britain and Ireland, residing at 51 Shooter's Hill road, 5 Blackheath, in the county of Kent, England, have invented certain new and useful Improvements in Explosives, of which the following is a specification.

My invention relates to nitroglycerin-nitrocellulose explosives for blasting purposes, and is especially applicable to explosives which are not sufficiently rapid in their detonation to be used with small detonators.

The object of the invention is to add to 15 such explosives ingredients which will increase their quickness of detonation and render it possible to use the explosives with small detonators.

The invention consists in adding to a nitro-glycerin-nitrocellulose explosive about five per cent. of a mixture containing ammonium perchlorate seventy-eight parts and sulfur twenty-two parts. In preparing the explosives according to my invention the nitro-glycerin-nitrocellulose jelly is incorporated 25 with the other constituents usually added for the purpose of moderating the explosive properties, and the mixture of sulfur and ammonium perchlorate is at the same time incorporated. The proportion of the mixture used will depend on the explosive properties 30 of the nitroglycerin-nitrocellulose powder to which it is added.

I find that with explosives whose properties are suitable for blasting practically all qualities of rock about five per cent. of the sulfur and perchlorate mixture is a convenient quantity to use. With the explosive so manufactured I find that detonators containing 40 about .5 gram of fulminate are sufficient to give excellent results.

As an example of an explosive according to my invention the following composition may be given:

|     |                                  |           |     |
|-----|----------------------------------|-----------|-----|
| (a) | Nitroglycerin . . . . .          | 495 parts | 45  |
|     | Soluble nitrocellulose . . . . . | 23 parts  |     |
|     | Pitch . . . . .                  | 6 parts   |     |
|     | Sodium nitrate . . . . .         | 52 parts  |     |
| (b) | Sodium nitrate . . . . .         | 140 parts | 95% |
|     | Woodmeal . . . . .               | 60 parts  |     |
| (c) | Sodium nitrate . . . . .         | 352 parts |     |
|     | Pitch . . . . .                  | 48 parts  |     |
| (d) | Ammonium perchlorate . . . . .   | 78 parts  | 5%  |
|     | Sulfur . . . . .                 | 22 parts  |     |

In preparing the explosive according to my invention the nitroglycerin jelly is preferably prepared by standing nitroglycerin in troughs until it is heated to about 120° Fahrenheit. The nitrocellulose is then added, the mixture being continually stirred until thoroughly mixed, while the pitch and sodium nitrate required to make up the mixture *a* are stirred in at the same time. The mixtures *b*, *c*, and *d* are then separately added to the jelly and the whole incorporated in any known form of incorporating-machine.

The composition of explosive given above is one suitable for blasting rocks of medium toughness, and it will be found that the explosive can be detonated successfully by about 0.5 gram of fulminate.

Having now described my invention, what I claim as new, and desire to secure by Letters Patent, is—

A nitroglycerin-nitrocellulose explosive, 75 containing about five per cent. of a mixture of ammonium perchlorate seventy-eight parts, and sulfur twenty-two parts, as and for the purposes described.

In testimony whereof I affix my signature 80 in presence of two witnesses.

OSWALD SILBERRAD.

Witnesses:

JOHN W. ADAMS,  
BERTRAM H. MATTHEWS.